

Dec. 16, 1947.

W. H. DIMSDALE ET AL

2,432,864

PHOTOGRAPHIC ELEMENTS BEARING SILVER HALIDE EMULSION LAYER AND ADJACENT  
LIGHT-INSENSITIVE COLLOID LAYER CONTAINING SILVER DERIVATIVES OF AZOLES

Filed Jan. 18, 1945

FIG. 1.



FIG. 2.



FIG. 3.



FIG. 4.



INVENTORS  
WILFRID HAMPDEN DIMSDALE  
and RICHARD ROBERT ROBINSON  
BY

*Lynn Barrett Morris*

ATTORNEY

## UNITED STATES PATENT OFFICE

2,432,864

## PHOTOGRAPHIC ELEMENTS BEARING SILVER HALIDE EMULSION LAYER AND ADJACENT LIGHT-INSENSITIVE COLLOID LAYER CONTAINING SILVER DERIVATIVES OF AZOLES

Wilfrid Hampden Dimsdale and Richard Robert Robinson, Ilford, England, assignors to Ilford Limited, Ilford, England, a British company

Application January 18, 1945, Serial No. 573,460  
In Great Britain February 3, 1944

5 Claims. (Cl. 95—8)

1

This invention relates to photographic light-sensitive elements, to compounds which serve as improvers for photographic silver halide emulsions, and particularly to compounds which improve the quality of the developed photographic images obtained in such emulsions.

In the production of photographic images in silver halide emulsions, and particularly in the case of emulsions consisting primarily of silver chloride, the maximum image density obtainable is not always so great as may be desired. Moreover, the common practice of hot-glazing photographic prints tends to affect adversely the image colour, giving a poor quality black which has a "bronzed" appearance, and also reduces the effective maximum density obtainable in the image.

In British Patent No. 561,875 methods are described for improving the quality of the developed photographic images which comprise treating the emulsions with 5-mercaptop-tetrazoles. These compounds may be introduced into the emulsion itself, or into a subcoat, supercoat or backing layer, or they may be included in the wrapping materials used. Alternatively, the compounds may be applied in solution to the emulsion before or during development, e. g. by including them in the developing solution used. These compounds, so used, not only improve the maximum image density obtainable and serve as "anti-bronzing" agents, but also reduce the level of fog in the developed image. As stated in the said patent, compounds used to reduce the fog level frequently cause a serious reduction in the speed of the emulsion, and it is an advantage of the compounds described in the said patent that the reduction in speed which they cause is not serious. Nevertheless, in the case of many of the compounds, some reduction in speed is caused by their use, as indicated by the figures set out in Table I of the said patent.

There are other classes of compounds which serve to increase the maximum image density obtainable and serve as anti-bronzing agents, among which are 5-mercaptop-1,2,4-triazoles described in U. S. application No. 558,270. These compounds, when incorporated in the emulsion or developer also serve to decrease the fog level in the developed image, and also sometimes effect a decrease in the speed of the emulsions.

Whilst the method of using such compounds described in the said U. S. application Serial No.

2

558,270, filed October 11, 1944, does not lead to a loss in speed of the emulsion, since the compounds are not applied until the emulsion has already been developed, the method entails that 5 the user needs to employ special fixing, glazing or other solutions containing the compounds. It would clearly be an advantage for the manufacturer to be able to include the compound in the photosensitive element as marketed, providing 10 that its presence in such element did not unduly reduce the speed of the photo-sensitive emulsion.

The present invention is concerned with a method of including the compounds in the photo-sensitive element itself in a form such that 15 any tendency for the compound to reduce the speed of the photo-sensitive emulsion is reduced or eliminated.

According to this invention there is added to 20 a photographic emulsion or to a colloid medium other than the emulsion which forms a water-permeable layer in a photographic element including a silver halide emulsion layer, a silver derivative of a compound which, when added 25 in its free state, or in the state of its alkali-metal derivative, improves the quality of photographic images developed in such emulsion layers.

The term "added" is intended to mean that the silver derivative itself is added or that 30 reagents are added which react among themselves to form the silver derivative. The mere addition of the free compound or of its alkali-metal derivative to a silver halide emulsion with the consequent possible formation of some silver derivative by reaction with part of the silver of the emulsion itself is not included within the meaning of the term and does not give the same results as are obtained by the process of this invention.

40 The term "silver derivative" is intended to mean a derivative resulting from replacement of hydrogen in the said compound by silver.

In a preferred form of the invention the silver derivatives are added to colloid media which are 45 to be used for coating layers in contact with the silver halide emulsion layer or layers. For example, the silver derivative may be included in a supercoat layer, e. g., a colloid layer coated on top of the photographic emulsion layer and forming, for example, an outer layer of the element, or may be included in a subcoat layer, e. g., a colloid layer lying between a photographic emul-

sion layer and a support layer, or may be included in an inter-layer between two emulsion layers. It may, however, be present in other layers, for example a backing layer.

The photographic elements described in the preceding paragraphs are illustrated in the accompanying drawing wherein:

Fig. 1 is a cross section of a film bearing a silver halide emulsion layer and a superposed layer containing an anti-bronzing agent of the type described below;

Fig. 2 is a cross section of a similar film wherein the silver halide layer is outermost;

Fig. 3 is a cross section of a similar film wherein a colloid layer containing an anti-bronzing agent is disposed between two emulsion layers; and

Fig. 4 is a cross section of a modified film wherein the two layers are on opposite surfaces.

Referring more particularly to the drawing, in Fig. 1 a film support 1 is provided with a silver halide emulsion layer 2 on which there is disposed a water-permeable colloid layer 3 containing an anti-bronzing agent of the type disclosed below.

In Fig. 2 a film support 1 is provided with a water-permeable colloid layer 4 containing an anti-bronzing agent as herein disclosed on which there is disposed a silver halide emulsion layer 5.

The element of Fig. 3 consists of a film support 1 bearing silver halide emulsion layers 6 and 8, between which there is disposed a water-permeable colloid layer 7 containing an anti-bronzing agent as herein disclosed.

The element of Fig. 4 consists of a film support 1 bearing a silver halide emulsion layer 9 on one surface and having disposed on the other surface a water-permeable colloid layer 10 containing a herein disclosed anti-bronzing agent.

It is desirable, especially where the silver derivative is included in a supercoat or in the emulsion layer itself, that it should be in a very fine state of subdivision in the layer in which it is incorporated. Thus, a convenient method of use is to form the silver derivative *in situ* in the colloid medium in which it is to be dispersed, for example by the double decomposition of a soluble silver salt and an alkali-metal derivative of the compound in a gelatin medium.

The invention may be applied to all varieties of compound which are capable of improving the quality of the developed image and which will form silver derivatives.

The following are typical classes of compounds which may be used, as their silver derivatives, in accordance with this invention.

(a) Compounds of the type described in British Patent No. 561,875. These are 5-mercaptop tetrazoles and specific examples are:

1-phenyl-5-mercaptop-tetrazole  
1- $\alpha$ -naphthyl-5-mercaptop-tetrazole  
1- $\beta$ -naphthyl-5-mercaptop-tetrazole  
1-p-diethylamino phenyl-5-mercaptop-tetrazole  
1-o-methoxy phenyl-5-mercaptop-tetrazole  
1-p-chlor phenyl-5-mercaptop-tetrazole  
1-benzyl-5-mercaptop-tetrazole  
1-cyclohexyl-5-mercaptop-tetrazole  
1-methyl-5-mercaptop-tetrazole  
1-ethyl-5-mercaptop-tetrazole

(b) The 5-mercaptop-1,2,4-triazoles described in U. S. application Serial No. 558,270, referred to above. Specific examples of these are:

1,2-dimethyl-5-mercaptop-1,3,4-triazole  
1-ethyl-2-methyl-5-mercaptop-1,3,4-triazole

1-phenyl-2-methyl-5-mercaptop-1,3,4-triazole  
1-phenyl-5-mercaptop-1,3,4-triazole  
1-benzyl-5-mercaptop-1,3,4-triazole  
1-methyl-2-ethyl-5-mercaptop-1,3,4-triazole  
5 1-methyl-2-n-hexyl-5-mercaptop-1,3,4-triazole  
1-p-hydroxy phenyl-2-methyl-5-mercaptop-1,3,4-triazole  
1-p-amino phenyl-2-methyl-5-mercaptop-1,3,4-triazole  
10 1- $\alpha$ -naphthyl-2-phenyl-5-mercaptop-1,3,4-triazole  
2- $\alpha$ -naphthyl-5-mercaptop-1,3,4-triazole  
1,2-diphenyl-5-mercaptop-1,3,4-triazole

(c) Heterocyclic nitrogen compounds containing two nitrogen atoms in the ring and one, two or three sulphur atoms attached to carbon atoms which are in  $\alpha$ -position to the nitrogen atoms (compounds containing a single sulphur atom linked to a carbon atom which is  $\alpha$  to both nitrogen atoms are included but are generally less efficient). Examples of this class of compound are:

2,5-dimercapo-1,3,4-thiodiazole  
2-mercaptop-5-amino-1,3,4-thiodiazole  
25 1-mercaptop-4-hydroxy-phthalazine  
1,4-dimercapo-phthalazine  
2,5-dimercapo-3-methyl-1,3,4-thiodiazole  
2-hydroxy-4-mercaptop pyrimidine  
2,4-dimercapo-pyrimidine  
30 2,4-dimercapo-quinazoline  
Trithio barbituric acid

(d) Mercapto hydroxy diazoles, an example of which is:

35 2-mercaptop-4-phenyl-5-hydroxy-1,3,4-thiodiazole.

(e) Dimercapto monazoles, an example of which is:

40 2,4-dimercapo quinoline.

(f) Mono mercapto monazoles, examples of which are:

2-mercaptop-benzthiazole  
2-mercaptop-benzoxazole  
45 2-mercaptop-quinoline  
2-mercaptop-6,7-benzbenzthiazole (i. e., naphthothiazole)  
4-mercaptop-quinoline.

50 As already indicated, the invention is of particular importance in the case of photo-sensitive elements carrying photographic silver chloride emulsions, since such emulsions are normally more subject to "bronzing." It may, however, be applied to other silver halide emulsions, e. g., silver chlorobromide, silver bromide and silver iodobromide emulsions. The invention is of particular value in connection with the production of the so-called "contact" printing paper consisting of, or comprising, a silver halide emulsion in which the predominant halide is silver chloride, coated on a paper support.

The following examples illustrate the invention:

#### 65 EXAMPLE I

1 gram of 1-phenyl-2-methyl-5-mercaptop-1,3,4-triazole was dissolved in 3.6 ccs. of a 40% aqueous solution of sodium carbonate (cryst.).  
70 This solution was added to 250 ccs. of a 4.4% solution of gelatin (containing a small quantity of dispersing agent) and made up to 500 ccs. with water. 77.7 ccs. of a 1% aqueous solution of silver nitrate was added to 250 ccs. of a 4.4% solution 75 of gelatin (containing a small quantity of dis-

persing agent) and made up to 500 ccs. with water. The second solution was added to the first quickly and with vigorous stirring, the solutions being maintained at 85° to 90° F. The mixture was cooled to 80° F., a small amount of formaldehyde added and then, after standing, was coated at 80° F. as a supercoat (a) a standard silver bromide emulsion as used in ordinary "bromide printing paper," and (b) a standard silver chloride emulsion as used in ordinary "contact" or "gaslight" printing paper, the emulsion layers being carried on paper supports. Test samples of the dried coatings were exposed behind a density step wedge, developed and fixed. Some samples were dried normally and others were dried on a commercial hot-glazing machine.

Control samples, in which the triazole compound was omitted from the gelation supercoat, were similarly processed, and the speed and maximum image density ( $D_{max}$ ) were determined for the various samples. The results obtained were as set out in the following Table I:

Table I

|                  | Silver Bromide Coatings |                          |                      | Silver Chloride Coatings |                          |                      |
|------------------|-------------------------|--------------------------|----------------------|--------------------------|--------------------------|----------------------|
|                  | Speed                   | $D_{max}$ normally dried | $D_{max}$ hot-glazed | Speed                    | $D_{max}$ normally dried | $D_{max}$ hot-glazed |
| Control.....     | 100                     | 1.91                     | 1.73                 | 100                      | 1.87                     | 1.36                 |
| Test Sample..... | 45                      | 1.95                     | 2.05                 | 100                      | 1.90                     | 1.98                 |

The speed values given above are on an arbitrary scale, but are inversely proportional to the exposures necessary to produce an image of reflection density 1.0. It will be noted that no measurable loss in speed was caused in the case of the silver chloride emulsion coatings, but some decrease in speed occurred with the silver bromide emulsion coatings. However, a com-

5  
6  
and the results obtained were as set out in the following Table II:

Table II

|                  | Silver Bromide Coatings |                          |                      | Silver Chloride Coatings |                          |                      |
|------------------|-------------------------|--------------------------|----------------------|--------------------------|--------------------------|----------------------|
|                  | Speed                   | $D_{max}$ normally dried | $D_{max}$ hot-glazed | Speed                    | $D_{max}$ normally dried | $D_{max}$ hot-glazed |
| Control.....     | 100                     | 1.91                     | 1.73                 | 100                      | 1.87                     | 1.36                 |
| Test Sample..... | 71                      | 1.95                     | 2.06                 | 100                      | 1.89                     | 1.95                 |

These speed values are calculated as before. Again there is no measurable loss in speed in the case of the silver chloride emulsion coatings, but there is some loss in the case of the silver bromide emulsion coatings. However, a comparable test on the silver bromide material using a supercoat containing the free compound (i. e., not as the silver derivative) showed a speed value only 5% of that of the test sample of the above Table II.

25 The test samples in all cases showed a markedly less degree of bronzing, after hot-glazing, than the control.

It should be pointed out that the speed figures given in this example are not comparable with the speed figures given in Example I of British Patent No. 561,875, though the same compound is in use, for the reason that in the present case very much larger quantities of the compound have been taken in the examples and the emulsions used are different.

## EXAMPLE III

The general procedure of Examples I and II was followed using concentrations of 1 part of the silver derivative in 5000 parts of the gelatin supercoat solution, other compounds than those used in Examples I and II being selected. The results obtained are set out in Table III.

Table III

| Compound                             | Silver Bromide Coatings  |      |                      |      | Silver Chloride Coatings |      |                      |      |
|--------------------------------------|--------------------------|------|----------------------|------|--------------------------|------|----------------------|------|
|                                      | $D_{max}$ normally dried |      | $D_{max}$ hot-glazed |      | $D_{max}$ normally dried |      | $D_{max}$ hot-glazed |      |
|                                      | Control                  | Test | Control              | Test | Control                  | Test | Control              | Test |
|                                      |                          |      |                      |      |                          |      |                      |      |
| 2,4-di-mercapto pyrimidine.....      | 1.91                     | 1.94 | 1.70                 | 2.05 | 1.74                     | 1.86 | 1.46                 | 2.00 |
| 1-mercapto-4-hydroxyphthalazine..... | 1.83                     | 1.94 | 1.58                 | 1.99 | 1.75                     | 1.90 | 1.45                 | 1.98 |
| 2-mercapto-benzthiazole.....         | 1.83                     | 1.89 | 1.58                 | 1.94 | 1.75                     | 1.86 | 1.45                 | 1.97 |
| 2,4-dimercapto quinoline.....        | 1.82                     | 1.85 | 1.71                 | 1.90 | 1.80                     | 1.83 | 1.53                 | 1.86 |

parable test on the silver bromide material using a supercoat containing the free compound (i. e., not as the silver derivative) showed a speed value only 1% of the speed of the test sample of the above Table I. The test samples in all cases showed a markedly less degree of bronzing after hot-glazing than the control.

## EXAMPLE II

The procedure given in Example I was followed with the variations that the compound used was 1-phenyl-5-mercapto-tetrazole, it was dissolved in 5.0 ccs. of the sodium carbonate solution and the quantity of silver nitrate solution taken was 95.5 ccs. All other conditions remained the same

65  
In all cases such loss of speed as occurred due to the use of the silver derivative was much less than the loss incurred by the use of the free compounds. In all cases an increase in  $D_{max}$  was obtained and the bronzing effect shown on the hot-glazed control samples was substantially entirely avoided in the test samples.

## EXAMPLE IV

70 The silver derivative of 1-phenyl-5-mercapto tetrazole was prepared and added in finely divided condition to silver chloride and silver bromide emulsions, one part of the silver derivative being added per 1000 parts of emulsion. Tests were

made as before and gave the results set out in Table IV.

Table IV

|                  | Silver Bromide Coating          |                             | Silver Chloride Coating         |                             |
|------------------|---------------------------------|-----------------------------|---------------------------------|-----------------------------|
|                  | D <sub>max</sub> normally dried | D <sub>max</sub> hot-glazed | D <sub>max</sub> normally dried | D <sub>max</sub> hot-glazed |
| Control.....     | 1.86                            | 1.75                        | 1.85                            | 1.39                        |
| Test Sample..... | 1.90                            | 2.03                        | 1.91                            | 2.04                        |

The bronzed effect of the control samples, shown particularly on the hot-glazed samples, was substantially eliminated in the test samples and, though some loss in speed was caused by the addition of the silver derivative to the bromide emulsion, this loss was less than is caused by the addition of the free compound. An increase in D<sub>max</sub> was effected in all cases.

What we claim is:

1. A photographic element comprising a silver halide emulsion layer and, in contact therewith, a water-permeable light-insensitive colloid layer which contains a silver derivative of a compound selected from the class consisting of 5-mercaptop-tetrazoles, 5-mercaptop-1,3,4-triazoles, diazoles containing up to three sulphur atoms attached to carbon atoms which are in  $\alpha$ -positions to the cyclic nitrogen atoms, mercapto hydroxy diazoles, dimercapto monazoless and monomercapto monazoless.

2. A photographic element comprising a silver halide emulsion layer and an outer water-permeable light-insensitive colloid layer in contact with said emulsion layer, said outer layer containing a preformed silver derivative of a compound selected from the class consisting of 5-mercaptop-tetrazoles, 5-mercaptop-1,3,4-triazoles, diazoles containing up to three sulphur atoms attached to carbon atoms which are in  $\alpha$ -positions to the cyclic nitrogen atoms, mercapto hydroxy diazoles, dimercapto monazoless and mono mercapto monazoless.

3. A photographic element comprising a silver halide emulsion layer of which the predominant silver halide is silver chloride and, in contact therewith, a water-permeable light-insensitive colloid layer which contains a silver derivative of

a compound selected from the class consisting of 5-mercaptop-tetrazoles, 5-mercaptop-1,3,4-triazoles, diazoles containing up to three sulphur atoms attached to carbon atoms which are in  $\alpha$ -positions to the cyclic nitrogen atoms, mercapto hydroxy diazoles, dimercapto monazoless and mono mercapto monazoless.

4. A photographic element comprising a silver halide emulsion layer of which the predominant

10 silver halide is silver chloride and an outer water-permeable light-insensitive colloid layer in contact with said emulsion layer, said outer layer containing a silver derivative of a compound selected from the class consisting of 5-mercaptop-tetrazoles, 5-mercaptop-1,3,4-triazoles, diazoles containing up to three sulphur atoms attached to carbon atoms which are in  $\alpha$ -positions to the cyclic nitrogen atoms, mercapto hydroxy diazoles, dimercapto monazoless and mono mercapto monazoless.

15 5. A photographic element comprising a paper support carrying a silver halide emulsion layer and an outer water-permeable light-insensitive colloid layer in contact with said emulsion layer, said outer layer containing a silver derivative of a compound selected from the class consisting of 5-mercaptop-tetrazoles, 5-mercaptop-1,3,4-triazoles, diazoles containing up to three sulphur atoms attached to carbon atoms which are in  $\alpha$ -positions to the cyclic nitrogen atoms, mercapto hydroxy diazoles, dimercapto monazoless and mono mercapto monazoless.

35 WILFRID HAMPDEN DIMSDALE.  
RICHARD ROBERT ROBINSON.

## REFERENCES CITED

The following references are of record in the file of this patent:

40

## UNITED STATES PATENTS

| Number    | Name       | Date          |
|-----------|------------|---------------|
| 2,057,764 | Brunkens   | Oct. 20, 1936 |
| 2,066,099 | Dieterle   | Dec. 29, 1936 |
| 2,221,805 | Leermakers | Nov. 19, 1940 |
| 2,377,375 | Russell    | June 5, 1945  |

## FOREIGN PATENTS

| Number     | Country       | Date          |
|------------|---------------|---------------|
| 50 390,037 | Great Britain | Mar. 30, 1933 |